

July 26, 1927.

D. R. TULLIS

1,636,881

PROCESS FOR PURIFYING OR REFINING METALS AND ALLOYS

Filed Nov. 9, 1926



Inventor:  
David Ronald Tullis,  
by Labor Law,  
Attorneys.

# UNITED STATES PATENT OFFICE.

DAVID RONALD TULLIS, OF CLYDEBANK, SCOTLAND.

## PROCESS FOR PURIFYING OR REFINING METALS AND ALLOYS.

Application filed November 9, 1926, Serial No. 147,227, and in Great Britain November 11, 1925.

This invention relates to a process of purifying or refining aluminium and its alloys while in the molten state to remove therefrom dissolved gases or other impurities.

5 The invention consists in introducing into the molten metal or alloy a gas containing chlorine, namely boron trichloride.

In practice chlorine gas is led through a desiccator and thence through a tube located 10 within a furnace and containing boron trioxide and carbon, so that there issue from the tube boron trichloride and carbon monoxide, whence the mixture passes through an absorbent for the carbon monoxide, and 15 the boron trichloride is led into a molten bath of aluminium alloy in which is a stirring device. As the gas is liberated in the bath, the boron passes into alloying relation with the aluminium and the chlorine expels 20 the gases contained in the alloy with the subsequent formation of aluminium chloride which rises to the top of the bath.

When it is ascertained that dissolved gases and/or other impurities are removed, the 25 metal or alloy may be transferred to moulds for the production of castings.

The figure of the accompanying drawing illustrates a simple form of apparatus suitable for the performance of the process.

As shown, 1 denotes a bottle charged with dry chlorine gas which is led from the bottle through a tube 2 located within a furnace 3 and containing say boron trioxide and carbon, so that there issue from the tube 2 boron trichloride and carbon monoxide, whence the mixture passes to the vessel 4 containing an absorbent for the carbon monoxide. From the vessel 4 the boron trichloride is led to the crucible 5 containing a molten charge of aluminium alloy by way of a tube 6 of silica 40 operatively connected by gearing to a motor 7 so that the tube may function as a stirrer. As the gas is liberated in the bath, the boron passes into alloying relation with the aluminium and the chlorine expels the gases 45 contained in the alloy with the subsequent formation of aluminium chloride which rises to the top.

I claim:—

A process of purifying or refining aluminium and its alloys consisting in introducing into the metal or alloy boron trichloride.

In testimony whereof I have signed my name to this specification.

DAVID RONALD TULLIS.